

Patented Nov. 23, 1926.

1,607,959

# UNITED STATES PATENT OFFICE.

BERNARD LOEWE, OF ZURICH, SWITZERLAND.

## METHOD OF REELING-OFF SILK COCOONS.

No Drawing. Application filed December 27, 1923, Serial No. 683,081, and in Austria January 24, 1923.

According to the present invention the cocoons are immersed in a bath consisting of an alkaline solution or a solution of alkaline earths (either in a caustic state or in combination with weak acids), the temperature of which is the same as the ordinary room temperature or lower, but may also be below freezing point. The time of immersion depends on the concentration and the temperature of the bath. According to the composition of the bath used albuminates are formed with the bast of the cocoon threads, which albuminates are insoluble in cold water, but soluble in hot water. The bast is thereby rendered soft and sticky, the threads of a number of cocoons treated at the same time adhere together and the reeling-off of the cocoon threads, from which the bast has not been removed, then proceeds easily in cold water or in a moist state in the air.

The scouring of the reeled-off silk (Grèges or twisted silk) can be subsequently effected in a simple manner before dyeing by a treatment in hot water in contradistinction to the usual reeling-off methods, in which the scouring is effected by the use of alkaline baths, soap, soap-suds or the like.

The treatment of cocoons according to the present invention may be carried out for instance in the following manner:

(1) Preferably the cocoons are first immersed in a cold bath consisting of neutral, alkaline or acid salts, mineral or organic acids or oils emulsified with or dissolved in alcohol or ether or sulphonated oils, according to the properties which it is desired to impart to the reeled-off threads (Grèges or twisted silk). The object of this treatment is to weaken the direct effect on the cocoon threads of the alkaline solutions or the solutions of alkaline earths used subsequently, by making the action indirect only. For preliminary baths of this kind substances may for instance be used, such as sodium acetate, sodium formate, zinc acetate, ammonium sulphate, magnesium sulphate, sodium chloride, zinc chloride, hydrochloric acid, acetic acid, lactic acid, formic acid, oleic acids and the like. The cocoons can be left immersed, for instance for 15 minutes or for a number of hours, according to the degree of concentration of this preliminary bath, while vacuum or pressure may be used for accelerating the action.

By this preliminary treatment the pupæ

of the silk-worms in the cocoons are killed and, when this has taken place, the cocoons may be stored for any length of time after being dried, before being subjected to further treatment and reeled-off. The cocoons can then be reeled-off by any of the well-known methods. According to the present invention this is effected in the following manner:

(2) Immediately after the cocoons have been treated in the bath referred to in paragraph (1) or after a short or long period, the cocoons are either washed or not washed or neutralized if necessary, after which they are immersed in a bath, which, as stated above, consists of an alkaline solution or a solution of alkaline earths, in a caustic state or in combination with weak acids, such as carbon dioxide, salicylic acid or the like. For this purpose for instance a solution of caustic soda of 0-3° Bé. or more, at a temperature of 25° C. or less, even below 0°, is used. The time of immersion is 1 to 30 minutes, but can be extended for several hours according to the degree of concentration and the temperature of the bath.

Fatty oils or soap may be added to this bath, which substances are suitable for reducing or increasing the action of the bath. In order to ensure that the solution should penetrate into all the hollow spaces within the cocoons, the work may be carried out at a pressure below or above that of the atmosphere. The bast fibres of the cocoon will thereby be softened right down to the innermost layers and the subsequent reeling-off of the cocoon can be effected without any difficulty. The threads of a number of cocoons will adhere to each other perfectly.

It may be remarked that the treatment described in paragraph (2) may be carried out alone, that is, without the preliminary treatment described in paragraph (1).

(3) The cocoons are thereupon bruised either in cold water or while they are still in the bath just described, in which they have been treated, so that the ends of the cocoons may be found and the cocoons may be reeled-off in cold water, without scouring them. The scouring can be effected subsequently in the finished Grèges or in the twisted thread by a simple treatment in boiling water, the reeled-off silk being for instance immersed for about 30 minutes in water at 100° C.

For increasing the lustre, the flexibility,

the elasticity and the toughness of the threads, substances, such as oil, glycerine, glucose or the like may be added to the baths, in which the cocoons have been treated.

Finally, the cocoons may be dyed before being reeled-off by immersing them, after they have passed through the chemical treatment described above, in a suitable dyeing 10 bath of the required shade. They are left in this bath until the dye has penetrated into all the hollow spaces, vacuum or pressure being used if required. The silk dyed in this manner has not been scoured and can 15 be softened during the dyeing of the cocoons by the addition of for instance oils or the like. The cocoons are thereupon rinsed in cold water or a slightly acidulated bath, after which the reeling-off and spinning may 20 be proceeded with. According to the way the spinning is carried out dyed Grèges or twisted silk is obtained in this manner.

What I claim is:—

1. A method of treating silk worm cocoons 25 without degumming consisting in first treating the cocoons in a preliminary bath of mainly a cold watery solution of at least one substance containing an acid radical, continuing this preliminary bath until the

silk worm pupae are killed, and then treating the cocoons in a second water bath containing an alkaline reacting substance for at least a minute at a temperature not exceeding 25° C., then reeling off the cocoons at an ordinary temperature, without the 30 employment of hot water, whereby the degumming can subsequently take place in ordinary hot water, without the addition of soap.

2. A method of treating silk cocoons as 40 claimed in claim 1 in which the treatment in the baths is conducted at a pressure less than atmospheric pressure.

3. A method of treating silk cocoons as 45 claimed in claim 1 having the added step of washing and drying the cocoons and storing them away for a period of time between the first and second baths.

4. A method of treating silk cocoons as 50 claimed in claim 1 in which the baths contain substances such as glycerine, glucose and the like, capable of increasing the elasticity, suppleness and toughness of the silk filaments of the threads.

In testimony whereof I have affixed my 55 signature.

BERNARD LOEWE.